



US005776647A

**United States Patent** [19]

Kido et al.

[11] **Patent Number:** **5,776,647**[45] **Date of Patent:** **Jul. 7, 1998**[54] **NEGATIVELY CHARGEABLE TONER FOR DEVELOPING ELECTROSTATIC LATENT IMAGE**5,665,512 9/1997 Tsutsui et al. .... 430/110  
5,705,303 1/1998 Ichimura et al. .... 430/110[75] Inventors: **Kenichi Kido; Tetsuo Sano**, both of Amagasaki; **Yoshitaka Sekiguchi**, Amagasaki; **Hiroyuki Fukuda**, Kobe, all of Japan[73] Assignee: **Minolta Co. Ltd.**, Osaka, Japan[21] Appl. No.: **948,525**[22] Filed: **Oct. 9, 1997**[30] **Foreign Application Priority Data**Mar. 4, 1997 [JP] Japan ..... 9-049122  
Mar. 4, 1997 [JP] Japan ..... 9-049124  
Mar. 4, 1997 [JP] Japan ..... 9-049125[51] **Int. Cl.<sup>6</sup>** ..... **G03G 9/097**[52] **U.S. Cl.** ..... **430/110; 430/111**[58] **Field of Search** ..... 430/110, 111[56] **References Cited**

## U.S. PATENT DOCUMENTS

5,660,964 8/1997 Machida et al. .... 430/110

*Primary Examiner*—Roland Martin[57] **ABSTRACT**

The negatively chargeable toner of the present invention includes a boron compound expressed by the chemical structural formula (A):

wherein R<sub>1</sub> and R<sub>3</sub> respectively represent substituted or non-substituted aryl group, R<sub>2</sub> and R<sub>4</sub> respectively represent hydrogen atom, alkyl group, substituted or non-substituted aryl group, X represents a cation, and n is an integer of either 1 or 2; to improve charge rise characteristics and charging stability.**35 Claims, No Drawings**

## 1

**NEGATIVELY CHARGEABLE TONER FOR  
DEVELOPING ELECTROSTATIC LATENT  
IMAGE**

**BACKGROUND OF THE INVENTION**

1. Field of the Invention

The present invention relates to a toner for developing electrostatic latent images, and specifically relates to a negatively chargeable toner for use in digital type image forming apparatuses.

2. Description of the Related Art

Conventional image forming apparatuses are generally analog type image forming apparatuses such as used in copiers and the like wherein a document is illuminated by a light source and the light reflected from said document irradiates the surface of a photosensitive member so as to form an electrostatic latent image on the surface of said photosensitive member. Image forming apparatuses of the digital type are known wherein digitally written electrostatic latent image is developed by supplying a developer containing a toner to said latent image. Digital type image forming apparatuses have been practicalized in the forms of electro-photographic type facsimile apparatuses, digital copiers which form images based on image information read by an image reader, and printers using the output of computer terminals.

In image forming apparatuses of the digital type, an electrostatic latent image is formed in dot units on the surface of a negatively charged organic photosensitive member by digitally writing image data via irradiation of said surface by a laser beam or the like. This latent image is reverse developed by a negatively charged toner, and the obtained toner image is transferred onto a recording member and fused thereon to form a recorded image. The toner used in such digital type processes must have excellent dot reproducibility. That is, the toner must have a true reproducibility in dot units when developing an electrostatic latent image formed on the surface of a photosensitive member, and this reproducibility must not be reduced even after repeated use. To satisfy such characteristics, a toner must have excellent charge rise characteristics as well as excellent stability relative to charging. In the case of two-component developers, a toner is mixed with a carrier within the developing device so as to be triboelectrically charged; the toner must have charging characteristics such that a desired amount of charge is attained rapidly in a short mixing time, but thereafter the charge amount drops somewhat or does not increase even with additional mixing.

Known art for improving the negative charging characteristics of a toner is the addition of various negative charge controller agents. Negative charge controllers have different charging characteristics depending on the type of controller, and many are known to increase the amount of negative charge of a toner, such that simply adding a charge controller does not produce the aforesaid excellent charging stability.

**SUMMARY AND OBJECTS OF THE  
INVENTION**

An object of the present invention is to eliminate the aforesaid disadvantages by providing a negatively chargeable toner having excellent charge rise characteristics and excellent charge stability.

Another object of the present invention is to provide a negatively chargeable toner having the aforesaid excellent charging characteristics and excellent black color reproducibility.

## 2

Still another object of the present invention is to provide a negatively chargeable toner which does not produce density irregularities in solid black images.

Yet another object of the present invention is to provide a negatively chargeable toner which eliminates the problem of reduced image quality caused by heat fixing by suppressing dot breakdown during heat fixing.

A further object of the present invention is to provide a negatively chargeable toner having excellent charge stability relative to environmental fluctuations.

A still further object of the present invention is to provide a negatively chargeable toner having excellent transfer characteristics from an electrostatic latent image carrying member such as a photosensitive member or the like to a transfer member such as a paper sheet or the like.

The present invention relates to a negatively chargeable toner comprising:

negatively chargeable toner particles including a binder resin, a colorant, an boron compound; wherein said binder resin includes a polyester resin and has an acid value of 5 to 50 KOHmg/g, and said colorant is carbon black having a pH of 1 to 6, and said boron compound is expressed by the chemical structural formula (A) below:



35 (Wherein R<sub>1</sub> and R<sub>3</sub> respectively represent substituted or non-substituted aryl group, R<sub>2</sub> and R<sub>4</sub> respectively represent hydrogen atom, alkyl group, substituted or non-substituted aryl group, X represents a cation, and n is an integer of either 1 or 2.)

40 The present invention relates to a negatively chargeable toner comprising:

negatively chargeable toner particles including a binder resin having an acid value of 5 to 50 KOHmg/g, a colorant, and a boron compound expressed by the chemical structural formula (A) below:



55 (Wherein R<sub>1</sub> and R<sub>3</sub> respectively represent substituted or non-substituted aryl group, R<sub>2</sub> and R<sub>4</sub> respectively represent hydrogen atom, alkyl group, substituted or non-substituted aryl group, X represents a cation, and n is an integer of either 1 or 2.); and

and exterior additive particles adhered to the toner particle surface, said exterior additive particles comprising hydrophobic silica particles and hydrophobic titanium dioxide particles, wherein the additive weight ratios of said hydrophobic silica particles and hydrophobic titanium dioxide particles is within a range of 10:1~1:10, the exterior additive total specific surface area S is 40~130 expressed by the equation (1) below:

$$S = S_s \times V_s + S_t \times V_t$$

(1)

(Wherein  $S_s$  is the specific surface area of the hydrophobic silica ( $m^2/g$ ),  $V_s$  is the additive amount (percent-by-weight; hereinafter abbreviated as "wt %") of hydrophobic silica particles relative to toner particles,  $S_t$  is the specific surface area of the hydrophobic titanium dioxide ( $m^2/g$ ), and  $V_t$  is the additive amount (percent-by-weight; hereinafter abbreviated as "wt %") of hydrophobic titanium dioxide particles relative to toner particles.

#### DESCRIPTION OF THE PREFERRED EMBODIMENTS

The negatively chargeable toner of the present invention includes a boron compound expressed by the chemical structural formula (A) below to improve charge rise characteristics and charging stability.



In the equation,  $R_1$  and  $R_3$  respectively represent substituted or non-substituted aryl group,  $R_2$  and  $R_4$  respectively represent hydrogen atom, alkyl group, substituted or non-substituted aryl group.  $X$  represents a cation, and  $n$  is an integer of either 1 or 2.

The previously described excellent effectiveness is accomplished by the inclusion of the aforesaid boron compound in a toner containing specific binder resin and specific colorant. That is, the toner has excellent negative chargeability before the inclusion of the boron compound, and is capable of maintaining a high negative charge. On the other hand, since this toner characteristically increases the amount of charge when mixed excessively, the inclusion of the aforesaid boron compound is believed to be effective in achieving excellent charging stability. The boron compound expressed by the chemical structural formula (A) has excellent safety characteristics inasmuch as it does not contain heavy metal.

Examples of usable cations represented by  $X$  in the aforesaid structural formula (A) include alkali metal ions such as lithium, potassium and the like, alkali earth metal ions such as magnesium, calcium and the like, hydrogen ion, ammonium ion, iminium ion, phosphonium ion and the like. The aforesaid boron compound is desirably added at a rate of 0.5 to 5 parts-by-weight, and preferably 1 to 3 parts-by-weight relative to 100 parts-by-weight (hereinafter parts-by-weight abbreviated to pbw) of binder resin. When the added amount of boron compound is less than 0.5 pbw, inadequate effectiveness is achieved, whereas when the added amount is in excess of 5 pbw, the amount of toner charge is reduced, causing the carrier to become spent too quickly when used in two-component developers.

In the present invention, it is desirable that the amount of the aforesaid boron compound present on the surface of the toner particle is 0.05 to 0.4 wt %, and preferably 0.1 to 0.3 wt %. The presence of the boron compound in the aforesaid amount on the surface of the toner provides adequate improvement of the toner charge rise characteristics as well as suitable effectiveness in improving charging stability. When the surface amount of said boron compound exceeds 0.4 wt %, the negative charge amount of the toner is reduced, and fogging readily occurs in the non-image region. The

amount of the boron compound present on the surface of the toner particles was measured by dispersing toner in a solvent capable of dissolving the boron compound so as to dissolve the boron compound present the toner particle surface, and subsequently separating the liquid, and assaying the boron compound (or one component thereof) in the liquid via atomic absorption photometry, ultraviolet absorption, fluorescence X-ray and the like. In the present invention, it is desirable that particles of the boron compound used is adjusted to a volume-average particle size of 5 to 25  $\mu m$ , and preferably 10 to 20  $\mu m$ , and it is further desirable that the content of said boron compound is 0.5 to 5 pbw, and preferably 1 to 4 pbw, relative to 100 pbw of binder resin.

Boron compounds possessing excellent characteristics will be colorless or white in color and, therefore disadvantageously reduce the degree of blackness of black toners. For example, the degree of blackness of the toner is reduced when using the aforesaid boron compound in place of azo compounds containing heavy metals such as chrome and cobalt and the like which are normally used as negative charge controllers because their color is black or a near-black dark color.

In the present invention, an acidic carbon black having a pH of 1 to 6, and preferably pH of 1 to 5, and more preferably pH of 1 to 4, so as to eliminate the aforesaid disadvantages. Such an acidic carbon black improves the degree of blackness by have excellent dispersibility relative a polyester resin having a specific acid value as described later. This carbon black also enhances the negative chargeability of the toner. Effectiveness is inadequate when an alkaline carbon black is used, and a reduced degree of blackness results using identical amounts compared to the use of acidic carbon black. The acidic carbon black content is desirably 6 to 12 pbw, and preferably 7 to 10 pbw relative to 100 pbw of binder resin. When the carbon black content is less than 6 pbw, inadequate effectiveness is achieved, whereas when more than 12 pbw are used, the toner charge is reduced so as to give rise to the disadvantages of toner fog and toner spillage. From the perspective of safety, it is desirable that the aforesaid carbon black should have a mean primary particle size of less than 40 nm, preferably 10 to 40 nm, and more preferably 15 to 35 nm.

The toner of the present invention desirably uses a binder resin including a polyester resin as the main component of the binder resin and having an acid value of 5 to 50 KOHmg/g, and preferably 10 to 40 KOHmg/g. Use of a binder resin having such an acid value improves the dispersibility of carbon black and boron compound, and produces a toner having sufficient negative charge. When the acid value is less than 5 KOHmg/g, the effectiveness is markedly reduced, and when the acid value exceeds 50 KOHmg/g, the stability of the toner charge amount is adversely affected by environmental fluctuations, especially temperature fluctuations.

The polyester resin used in the present invention may be a polyester resin obtained by a condensation polymerization reaction of a polyvalent alcohol component and polyvalent carboxylic acid component.

Examples of useful bivalent alcohol components among the aforesaid polyvalent alcohol components include bisphenol-A alkylene oxide adducts such as polyoxypolypropylene(2.2)-2,2-bis(4-hydroxyphenyl)propane, polyoxypolypropylene(3.3)-2,2-bis(4-hydroxyphenyl)propane, polyoxypolypropylene(6)-2,2-bis(4-hydroxyphenyl)propane, polyoxypolyethylene(2.0)-2,2-bis(4-hydroxyphenyl)propane and the like, ethylene glycol, triethylene glycol, 1,2-propylene glycol, 1,3-propylene glycol, 1,4-butanediol, neopentyl glycol, 1,4-butanediol, 1,5-pentanediol, 1,6-

hexanediol, 1,4-cyclohexane dimethanol, dipropylene glycol, polyethylene glycol, polytetramethylene glycol, bisphenol-A, bisphenol-A with added hydrogen and the like.

Examples of useful trivalent and above alcohol components include sorbitol, 1,2,3,6-hexanetetrol, 1,4-sorbitane, pentaerythritol, dipentaerythritol, tripentaerythritol, 1,2,4-butanetriol, 1,2,5-pantanetriol, glycerol, 2-methylpropanetriol, 2-methyl-1,2,4-butanetriol, trimethylolethane, trimethylolpropane, 1,3,5-trihydroxymethylbenzene and the like.

Examples of useful bivalent carboxylic acid components among the aforesaid polyvalent carboxylic acid component include maleic acid, fumaric acid, citraconic acid, itaconic acid, glutamic acid, phthalic acid, isophthalic acid, terephthalic acid, cyclohexane dicarboxylic acid, succinic acid, adipic acid, sebatic acid, azelaic acid, malonic acid, n-dodecylsuccinic acid, isododecylsuccinic acid, n-dodecylsuccinic acid, isododecylsuccinic acid, n-octenylsuccinic acid, isoctenylsuccinic acid, n-octylsuccinic acid, isoctylsuccinic acid, and acid anhydrides or low-molecular alkyl esters thereof.

Examples of useful trivalent and above carboxylic acid components include 1,2,4-benzenetricarboxylic acid, (trimellitic acid), 1,2,5-benzenetricarboxylic acid, 2,5,7-naphthalenetricarboxylic acid, 1,2,4-naphthalenetricarboxylic acid, 1,2,4-butanetricarboxylic acid, 1,2,5-hexanetricarboxylic acid, 1,3-dicarboxyl-2-methyl-2-methylenecarboxy propane, 1,2,4-cyclohexanetricarboxylic acid, tetra(methylecarboxyl)methane, 1,2,7,8-octane tetra-carboxylic acid, pyromellitic acid, empol trimer acid, and acid anhydrides and low-molecular alkyl esters thereof.

The binder resin used in the present invention may be a resin obtained by parallel reactions in the same vessel comprising a radical polymerization reaction of vinyl resin and a condensation polymerization reaction of a polyester resin using a raw monomer of polyester resin, raw monomer of vinyl resin and dual-reactive monomer. The dual-reactive monomer is a raw monomer that can use the dual reactions of the condensation polymerization and the radical polymerization. That is, the dual-reactive monomer has a carboxy group for the condensation polymerization and a vinyl group for the radical polymerization, e.g., fumaric acid, maleic acid, acrylic acid, methacrylic acid and the like.

The raw monomers of the polyester resin may have the aforesaid polyvalent alcohol component and polyvalent carboxylic acid component.

Examples of useful raw monomers of vinyl resin include styrene or styrene derivatives such as styrene, o-methylstyrene, m-methylstyrene, p-methylstyrene,  $\alpha$ -methylstyrene, p-ethylstyrene, 2,4-dimethylstyrene, p-tert-butylstyrene, p-chlorostyrene and the like; ethylene unsaturated monoolefins such as ethylene, propylene, butylene, isobutylene and the like; alkyl ester methacrylates such as methylmethacrylate, n-propylmethacrylate, isopropylmethacrylate, n-butylmethacrylate, isobutylmethacrylate, t-butylmethacrylate, n-pentylmethacrylate, isopentylmethacrylate, neopentylmethacrylate, 3-(methyl)butylmethacrylate, hexylmethacrylate, octylmethacrylate, nonylmethacrylate, decylmethacrylate, undecylmethacrylate, dodecylmethacrylate and the like; alkyl ester acrylates such as methylacrylate, n-propylacrylate, isopropylacrylate, n-butylacrylate, isobutylacrylate, t-butylacrylate, n-pentylacrylate, isopentylacrylate, neopentylacrylate, 3-(methyl)butylacrylate, hexylacrylate, octylacrylate, nonylacrylate, decylacrylate, undecylacrylate, dodecylacrylate and the like; and acrylonitrile, maleic acid ester, itaconic acid ester,

vinylchloride, vinyl acetate, vinylbenzoate, vinylmethyl-ethyl ketone, vinylhexyl ketone, vinylmethyl ether, vinyl-ethyl ether, vinylisobutyl ether and the like. Examples of useful polymerization initiators when polymerizing the raw monomers of vinyl resin include azo and diazo polymerization initiators such as 2,2'-azobis(2,4-dimethylvaleronitrile), 2,2'-azobisisobutyronitrile, 1,1'-azobis(cyclohexane-1-carbonitrile), 2,2'-azobis-4-methoxy-2,4-dimethylvaleronitrile and the like; and peroxide polymerization initiators such as benzoylperoxide, methylethylketone peroxide, isopropyl peroxycarbonate, lauroyl peroxide and the like.

In the present invention, it is desirable that the binder resin comprise two types of resins having different softening points so as to improve fixing characteristics, and to improve anti-offset characteristics. That is, it is desirable that a first resin having a softening point of 95° to 120° C. is used to improve fixing characteristics, and a second resin having a softening point of 130° to 160° C. is used to improve anti-offset characteristics. In this case, when the softening point of the first resin is less than 95° C., anti-offset characteristics are reduced and cause a reduction in dot reproducibility, and when the softening point is in excess of 120° C., there is inadequate improvement of fixing characteristics. When the softening point of the second resin is less than 130° C., there is inadequate improvement of anti-offset characteristics, and when the softening point is in excess of 160° C., fixing characteristics are reduced. From these perspectives, therefore, it is desirable that the softening point of the first resin is 100° to 115° C., and the softening point of the second resin is 135° to 155° C. It is further desirable that the glass transition temperatures of the first and second resins is 50° to 75° C., and preferably 55° to 70° C. When the glass transition temperature is less than 55° C., the toner has inadequate heat resistance, whereas when the glass transition temperature is higher than 70° C., pulverization characteristics during manufacture are lowered and cause a reduction in production efficiency.

It is desirable that the aforesaid first polyester resin should be a polyester resin produced by condensation polymerization of the aforesaid polyvalent alcohol component and polyvalent carboxylic acid component, and it is particularly desirable that the polyester resin has bisphenol-A alkylene oxide additive as a main polyvalent alcohol component, and at least one polyvalent carboxylic acid monomer selected from the group consisting of terephthalic acid, fumaric acid, dodecylsuccinic acid, benzenetricarboxylic acid as a main polyvalent carboxylic acid component.

From the perspectives of improving wax dispersibility, toner strength, fixing characteristics, and anti-offset characteristics is desirable that the second resin should be the resin obtained by parallel reactions in the same vessel comprising the radical polymerization reaction of vinyl resin and the condensation polymerization reaction of a polyester resin using the raw monomer of polyester resin, the raw monomer of vinyl resin and the dual-reactive monomer. The vinyl resin content of the second resin is desirably 5 to 40 percent-by-weight, and preferably 10 to 35 percent-by-weight (hereinafter percent-by-weight is abbreviated to wt %). When the vinyl resin content is less than 5 wt %, polyethylene wax dispersibility is reduced, and toner fixing strength is reduced. When the vinyl resin content exceeds 40 wt %, polypropylene wax dispersibility is reduced, and anti-offset characteristics and toner strength are reduced, and lead to low negative charge level in the toner.

The weight ratio of the first resin to the second resin is desirably 7:3 to 2:8, and preferably 6:4 to 3:7. Using first and

second resins within the aforesaid ranges produces excellent dot reproducibility by minimizing toner breakdown during fixing, and maintains excellent fixing characteristics even in image forming apparatuses operating at low and high speeds by having excellent low temperature fixing characteristics. Furthermore, excellent dot reproducibility is maintained even in the case of forming images on both sides of a sheet (i.e., passing through the fixing device twice). When the ratio of the first resin is less than the aforesaid range, low temperature fixing characteristics are inadequate and a broad range of fixing characteristics cannot be assured. When the ratio of the second resin is less than the aforesaid range, anti-offset characteristics are reduced, and dot reproducibility is tends to be reduced due to toner breakdown during fixing. The softening point of the resin was determined using a flow tester (model CFT-500; Shimazu Seisakusho); the softening point was designated as the temperature corresponding to  $\frac{1}{2}$  the height from the flow start point to the flow end point when a  $1\text{ cm}^3$  sample was melted under conditions of die pore size of 1 mm diameter by 1 mm length, pressure of  $20\text{ kg/cm}^2$ , and temperature rise rate of  $6^\circ\text{ C./min}$ . The glass transition temperature was measured using a differential scanning calorimeter(model DCS-200; Seiko Denshi) and alumina as a reference; a 10 mg sample was heated from  $20^\circ$  to  $120^\circ\text{ C.}$  with a temperature rise rate of  $10^\circ\text{ C./min}$ , and the shoulder value at the main endothermic peak was designated the glass transition temperature. The acid value of the resin is the value calculated from the uptake of a N/10 sodium hydroxide/alcohol solution by titrating a previously standardized N/10 sodium hydroxide/alcohol solution using 0.1% bromothymol blue and phenol red mixed indicator with 10 mg of sample material dissolved in 50 ml toluene.

Wax may be included in the toner of the present invention to improve characteristics such as anti-offset characteristics. Examples of useful waxes include polyethylene wax, polypropylene wax, carnauba wax, rice wax, sasol wax, montan ester wax, fischer-tropsch wax and the like. When such wax is included in the toner, the wax content is desirably 0.5 to 5 pbw relative to 100 pbw of binder resin to achieve effectiveness in preventing filming and the like.

It is desirable to include polypropylene wax in the toner from the perspective of improving anti-offset characteristics. It is further desirable to include polyethylene wax in the toner from the perspective of improving smear characteristics (i.e., smearing occurs when is blurred or soiled by a roller when fed by an aut feeder or when making a duplex copy with an image already formed on one side of the sheet). A particularly desirable polypropylene wax, from the aforesaid perspectives, will have a melt viscosity of 50 to 300 cps at  $160^\circ\text{ C.}$ , a softening point of  $130^\circ$  to  $160^\circ\text{ C.}$ , and an acid value of 1 to 20 KOHmg/g. A particularly desirable polyethylene wax will have a melt viscosity of 1,000 to 8,000 cps at  $160^\circ\text{ C.}$ , and a softening point of  $130^\circ$  to  $150^\circ\text{ C.}$  The wax melt viscosity was measured using a Brookfield viscometer.

Magnetic powder or the like may be added to the toner of the present invention as necessary. Examples of useful magnetic powders include well-known fine magnetic particles such as ferrite, magnetite, iron and the like, and may be added from the perspective of preventing airborne dispersion of the toner. The amount of added magnetic powder is desirable 0.5 to 10 pbw, preferably 0.5 to 8 pbw, and more preferably 1 to 5 pbw, relative to 100 pbw of binder resin. When the amount of added magnetic powder exceeds 10 pbw, developing characteristics are reduced due to the strengthening of the magnetic flux force exerted the developer carrying member (within the magnet roller) on the toner.

The toner of the present invention may have an exterior coating of inorganic microparticles on its surface. The toner and inorganic microparticles may be subjected to mechanical mixing to achieve the surface coating.

- 5 Examples of useful inorganic microparticles include silica particles, titanium dioxide particles, alumina particles, magnesium fluoride particles, silicon carbide particles, boron carbide particles, titanium carbide particles, zirconium carbide particles, boron nitride particles, titanium nitride particles, zirconium nitride particles, magnetite particles, molybdenum disulfide particles, barium titanate particles, strontium titanate particles, aluminum stearate particles, magnesium stearate particles, zinc stearate particles and the like used individually or in combinations of two or more.
- 10 15 The amount of added inorganic microparticles is desirably 0.05 to 2 percent-by-weight, and preferably 0.1 to 1 percent-by-weight relative to the toner. The addition of the inorganic microparticles in the aforesaid amount improves flow characteristics without loss of environmental stability of the
- 20 25 developer. Furthermore, it is desirable from the perspective of improved environmental stability that the aforesaid inorganic microparticles are subjected to hydrophobic processing using, for example, silane coupling agent, titanium coupling agent, higher fatty acids, silicone oil and the like.
- 30 35 It is desirable that hydrophobic silica and hydrophobic titanium dioxide are used as exterior additive microparticles in the present invention. Hydrophobic silica and hydrophobic titanium dioxide in this instance mean silica and titanium dioxide subjected to surface treatment via a hydrophobic agent such as silane coupling agent, silicone oil or the like. Use of the hydrophobic silica and hydrophobic titanium dioxide improves charge stability relative to environmental fluctuations and prevents a loss of charge under high-temperature high-humidity conditions.

- 40 45 The additive weight ratios of the hydrophobic silica particles and hydrophobic titanium dioxide particles is desirably within a range of 10:1 to 1:10, and preferably 8:1 to 1:5, and the exterior additive total specific surface area S is 40 to 130, and preferably 50 to 100, expressed by the equation (1) below:

$$S = S_s \times V_s + S_t \times V_t \quad (1)$$

- (wherein  $S_s$  is the specific surface area of the hydrophobic silica ( $\text{m}^2/\text{g}$ ),  $V_s$  is the additive amount (wt %) of hydrophobic silica particles relative to toner particles,  $S_t$  is the specific surface area of the hydrophobic titanium dioxide ( $\text{m}^2/\text{g}$ ), and  $V_t$  is the additive amount (wt %) of hydrophobic titanium dioxide particles relative to toner particles). By adding hydrophobic silica and hydrophobic titanium dioxide in a specific weight ratio, i.e., at a specific total specific surface area, toner flow characteristics, toner charge stability relative to environmental fluctuations, and transfer characteristics from the photosensitive member to the transfer sheet are markedly improved and fogging is prevented during printing.

- 50 55 In the present invention, it is desirable that the hydrophobic silica have a BET specific surface area of 100 to 250 ( $\text{m}^2/\text{g}$ ), and preferably 120 to 200 ( $\text{m}^2/\text{g}$ ).

- 60 65 It is further desirable that the hydrophobic titanium dioxide have a BET specific surface area of 40 to 150 ( $\text{m}^2/\text{g}$ ), and preferably 80 to 130 ( $\text{m}^2/\text{g}$ ). From the perspective of flow characteristics, it is desirable that the titanium dioxide is an amorphous titanium dioxide or anatase titanium dioxide having a mean primary particle size of 10~70 nm. It is further desirable that the shape of the titanium dioxide particles are disk shaped from the perspective of adherence to the toner particles.

The toner particles in the present invention have a volume-average particle size of 3 to 9  $\mu\text{m}$ , and preferably 6 to 9  $\mu\text{m}$ , from the standpoint of high resolution image reproducibility.

The toner of the present invention may be used in a two-component developer together with a carrier, or in a monocomponent developer without a carrier. The carrier used in a two-component developer may be a well-known conventional carrier.

The present invention is described by way of experimental examples below, but is not limited to these experimental examples.

## Production of Polyester Resins L1-L3

Polyoxypolyethylene(2.2)-2,2-bis(4-hydroxyphenyl)propane, polyoxyethylene(2.2)-2,2-bis(4-hydroxyphenyl)propane, anhydrous isododecenylsuccinic acid, terephthalic acid, and fumaric acid were combined to achieve a weight ratio of 82:77:16:32:30. The mixture was introduced into a four-mouth flask to which a reflux condenser, nitrogen gas tube, thermometer, and mixing device were attached, then dibutyl tin oxide was added as a polymerization initiator. The material was heated in a mantle heater under a nitrogen atmosphere and reacted by mixing at 220° C. to obtain linear polyester resins L1-L3. The obtained polyester resin L1 had a softening point of 110° C., glass transition temperature of 60° C., and acid value of 17.5 KOHmg/g. The obtained polyester resin L2 had a softening point of 100° C., glass transition temperature of 52° C., and acid value of 19.3 KOHmg/g. The obtained polyester resin L3 had a softening point of 118° C., glass transition temperature of 73° C., and acid value of 15.9 KOHmg/g.

### Production of Polyester Resin L4

Polyoxypropylene(2.2)-2,2-bis(4-hydroxyphenyl)propane, polyoxyethylene(2.2)-2,2-bis(4-hydroxyphenyl)propane, terephthalic acid, and anhydrous 1,2,4-benzenetricarboxylic acid were combined to achieve a weight ratio of 73:30:45:3. The mixture was introduced into a four-mouth flask to which a reflux condenser, nitrogen gas tube, thermometer, and mixing device were attached, then dibutyl tin oxide was added as a polymerization initiator. The material was heated in a mantle heater under a nitrogen atmosphere and reacted by mixing at 220° C. The obtained polyester resin L4 had a softening point of 111.5° C., glass transition temperature of 70° C., and acid value of 19.3 KOHmg/g.

## Production of Polyester Resins H1–H3

Styrene and 2-ethylhexylacrylate were combined at a weight ratio of 17:3.2, and dicumyl peroxide was introduced via a titration rod as a polymerization initiator. Polyoxypropylene(2.2)-2,2-bis(4-hydroxyphenyl) propane, polyoxyethylene(2.2)-2,2-bis(4-hydroxyphenyl) propane, anhydrous isododecylsuccinic acid terephthalic acid, anhydrous 1,2,4-benzenetricarboxylic acid, and acrylic acid were combined to achieve a weight ratio of 42:11:11:11:8:1, and the mixture was introduced into a four-mouth flask to which a reflux condenser, nitrogen gas tube, thermometer, and mixing device were attached, then dibutyl tin oxide was added as a polymerization initiator. The material was mixed in a mantle heater under a nitrogen atmosphere at 135°C. as the styrene/2-ethylhexylacrylate solution was titrated in via the titration rod, and thereafter the temperature was elevated and the materials were reacted at 230°C. to obtain polyester resins H1–H3. The obtained polyester resin H1 had a softening point of 150°C., glass transition temperature of 62°C., and acid value of 24.5 KOHmg/g. The obtained polyester resin H2 had a softening point of 136°C., glass transition temperature of 52°C., and acid value of 26.3

KOHmg/g. The obtained polyester resin H3 had a softening point of 158°C., glass transition temperature of 73°C., and acid value of 21.4 KOHmg/g. The polyester resins H1–H3 were resins containing polyester resin and vinyl resin.

## 5 Production of Polyester Resin H4

Polyoxypropylene(2.2)-2,2-bis(4-hydroxyphenyl)propane, polyoxyethylene(2.2)-2,2-bis(4-hydroxyphenyl)propane, anhydrous isododecenylsuccinic acid, terephthalic acid, and anhydrous 1,2,4-benzenetricarboxylic acid were combined to achieve a weight ratio of 73:30:18:25:3. The mixture was introduced into a four-mouth flask to which a reflux condenser, nitrogen gas tube, thermometer, and mixing device were attached, then dibutyl tin oxide was added as a polymerization initiator. The material was heated in a mantle heater under a nitrogen atmosphere and reacted by mixing at 220° C. The obtained polyester resin H4 had a softening point of 154° C., glass transition temperature of 64° C., and acid value of 20.4 KOHmg/g.

## EXPERIMENTAL EXAMPLE 1

A mixture of 40 pbw polyester resin L1, 60 pbw polyester resin H1, 2 pbw polyethylene wax (400P; Mitsui Sekiyu Kagaku Kogyo; melt viscosity 1600 cps at 160° C., softening point: 136° C.), 2 pbw polypropylene wax (Biscol 550P; Sanyo Kasei Kogyo; melt viscosity of 200 cps at 160° C., softening point: 150° C.), 8 pbw acidic carbon black (MA77; Mitsubishi Chemicals; pH3, mean primary particle size: 23 nm), and 2 pbw negative charge controller having the chemical structural formula below



were added to a Henschel mixer and thoroughly mixed. The obtained mixture was fusion kneaded using a twin-shaft extrusion kneader, then cooled. The cooled mixture was 45 coarsely pulverized using a hammer mill, and the coarsely pulverized material was finely pulverized using a jet mill, and then the material was then classified to obtain toner particles having a volume-average particle size of 7.5  $\mu\text{m}$ .

These toner particles were mixed with 0.4 wt % hydrophobic silica microparticles having a BET specific surface area of 140 m<sup>2</sup>/g (H2000; Hoechst), and 0.2 wt % hydrophobic titanium dioxide microparticles having a BET specific surface area of 110 m<sup>2</sup>/g (STT30A; Chitan Kogyo) to obtain the end toner.

## EXPERIMENTAL EXAMPLE 2

Toner was produced in the same manner as in Experimental example 1 with the exception that 60 pbw of polyester resin L1 and 40 pbw polyester resin H1 were used.

### EXPERIMENTAL EXAMPLE 3

Toner was produced in the same manner as in Experimental example 1 with the exception that 50 pbw polyester resin L4 was substituted for the polyester resin L1, 50 pbw polyester resin H4 was substituted for polyester resin H1, and Regal 400R (Cabot; pH4; mean primary particle size: 25 nm) was used as the carbon black.

## 11

## EXPERIMENTAL EXAMPLE 4

Toner was produced in the same manner as in Experimental example 1 with the exception that 10 pbw carbon black was used.

## EXPERIMENTAL EXAMPLE 5

Toner was produced in the same manner as in Experimental example 3 with the exception that Regal 330 (Cabot; pH9.0; mean primary particle size: 25 nm) was used as the carbon black.

## EXPERIMENTAL EXAMPLE 6

Toner was produced in the same manner as in Experimental example 3 with the exception that zinc salicylate complex salt E84 (Orient Chemical Industries) was used as a negative charge controller.

## EXPERIMENTAL EXAMPLE 7

Toner was produced in the same manner as in Experimental example 1 with the exception that 100 pbw styrene-acrylic resin (MX-9500; Sanyo Kasei Kogyo) was substituted for polyester resins L1 and H1.

## EXPERIMENTAL EXAMPLE 8

Toner was produced in the same manner as in Experimental example 3 with the exception that azo dye with iron T77 (Hodogaya Kagaku Kogyo) was used as a negative charge controller.

## EXPERIMENTAL EXAMPLE 9

Toner was produced in the same manner as in Experimental example 3 with the exception that calix arene compound E89 (Orient Chemical Industries) was used as a negative charge controller.

## EXPERIMENTAL EXAMPLE 10

Toner was produced in the same manner as in Experimental example 3 with the exception that quaternary ammonium salt with fluoride VP434 (Hoechst) was used as a negative charge controller.

## EXPERIMENTAL EXAMPLE 11

Toner was produced in the same manner as in Experimental example 3 with the exception that terpene diphenol compound YP90 (Yasuhaba Chemicals) was used as a negative charge controller.

Each of the aforesaid toners were mixed with a pure carrier at a toner-to-carrier weight ratio of 5:95 to produce developer which was used in a digital copier (model Di30; Minolta Co., Ltd.). The toners were evaluated and the evaluation results are shown in Table 1.

## Charge Rise Characteristics

Each of the aforesaid developers was loaded in a plastic bottle and rotated at 120 rpm on a ball mill table to mix for 5, 10, 30, 60, 120, and 780 minutes, after which the amount of charge was measured (under environmental conditions of 25° C., 45% relative humidity).

The amount of charge after 5 min relative to a maximum charge value {(amount of charge after 5 min/maximum charge value)×100} of 90% or greater was deemed an extraordinary excellent charge rise and designated by a rank of O. 80% and higher but less than 90% was deemed suitable for practical use and designated by a rank of Δ, and less than

## 12

80% was deemed unsuitable for practical use and designated by a rank of X.

## Charge Stability

In the aforesaid evaluation of charge rise characteristics, 5 a minimum charge value of 15 μC/g and higher but less than 25 μC/g was ranked O, a minimum charge value of 10 μC/g and higher but less than 15 μC/g was ranked Δ, and a minimum charge value of less than 10 μC/g was ranked X. Initial Fog and Post-printing Fog

10 Each of the developers was used to make 100,000 prints using a model Di30 digital copier, and the images were visually examined at initial printing (after 100 sheets) and at the end of printing. Images with no trace of fog were ranked O, images with slight fog that posed no practical problem were ranked Δ, and images with noticeable fog making them unsuitable for practical use were ranked X.

## Image blackness

15 Using the mode Di30 digital copier, solid images (2×2 cm) having 1.0 mg/cm<sup>2</sup> toner adhesion were formed, and the 20 formed images were visually inspected. Excellent blackness was ranked O, slight irregularity when light was transmitted through the sheet but which posed no practical problem was ranked Δ, and weak color even without light transmission through the sheet was ranked X.

TABLE 1

|       | Charge Rise | Charge Stability | Initial Fog | End Fog | Image Blackness |
|-------|-------------|------------------|-------------|---------|-----------------|
| Ex 1  | ○           | ○                | ○           | ○       | ○               |
| Ex 2  | ○           | ○                | ○           | ○       | Δ               |
| Ex 3  | ○           | ○                | ○           | ○       | Δ               |
| Ex 4  | ○           | Δ                | ○           | Δ       | ○               |
| Ex 5  | ○           | ✗                | ○           | Δ       | ✗               |
| Ex 6  | ✗           | Δ                | Δ           | ✗       | ✗               |
| Ex 7  | Δ           | ✗                | Δ           | ✗       | Δ               |
| Ex 8  | ✗           | Δ                | ○           | Δ       | ○               |
| Ex 9  | ✗           | ✗                | ✗           | ✗       | ✗               |
| Ex 10 | ✗           | ✗                | Δ           | ✗       | Δ               |
| Ex 11 | ✗           | ✗                | Δ           | ✗       | Δ               |

## EXPERIMENTAL EXAMPLE 12

40 A mixture of 40 pbw polyester resin L1, 60 pbw polyester resin H1, 1 pbw polyethylene wax (800P; Mitsui Sekiyu Kagaku Kogyo; melt viscosity 5400 cps at 160° C., softening point: 140° C.), 2 pbw polypropylene wax (TS-100; Sanyo Kasei Kogyo; melt viscosity of 120 cps at 160° C., softening point: 144° C.), 8 pbw carbon black (Black Pearls, L; Cabot; pH2.5, mean primary particle size: 24 nm), and 2 pbw boron compound having the chemical structural formula below



and adjusted via pulverization to a volume-average particle size of 15 μm were added to a Henschel mixer and thoroughly mixed. The obtained mixture was fusion kneaded using a twin-shaft extrusion kneader, then cooled. The cooled mixture was coarsely pulverized using a hammer mill, and the coarsely pulverized material was finely pul-

## 13

verized using a jet mill, and then the material was then classified to obtain toner particles having a volume-average particle size of 7.5  $\mu\text{m}$ .

These toner particles were mixed with 0.4 percent-by-weight hydrophobic silica microparticles having a BET specific surface area of 140  $\text{m}^2/\text{g}$  (H2000; Hoechst), and 0.2 percent-by-weight hydrophobic titanium dioxide microparticles having a BET specific surface area of 110  $\text{m}^2/\text{g}$  (STT30A; Chitan Kogyo) to obtain the end toner.

## EXPERIMENTAL EXAMPLE 13

Toner was produced in the same manner as in Experimental example 12 with the exception that the boron compound was change to material having a volume-average particle size of 8  $\mu\text{m}$ , and 6 pbw Monarch 1300 (Cabot; pH2.5; mean primary particle size: 13 nm) was used as carbon black.

## EXPERIMENTAL EXAMPLE 14

Toner was produced in the same manner as in Experimental example 12 with the exception that the boron compound was change to material having a volume-average particle size of 22  $\mu\text{m}$ , and 6 pbw Regal 400 (Cabot; pH4.0; mean primary particle size: 25 nm) was used as carbon black.

## EXPERIMENTAL EXAMPLE 15

Toner was produced in the same manner as in Experimental example 12 with the exception that 50 pbw polyester resin L2 was substituted for polyester resin L1, 50 pbw polyester resin H2 was substituted for polyester resin H1, and Mogul L (Cabot; pH2.5; mean primary particle size: 24 nm) was used as carbon black.

## EXPERIMENTAL EXAMPLE 16

Toner was produced in the same manner as in Experimental example 12 with the exception that 30 pbw polyester resin L3 was substituted for polyester resin L1, 70 pbw polyester resin H3 was substituted for polyester resin H1, and 12 pbw Mogul L (Cabot; pH2.5; mean primary particle size: 24 nm) was used as carbon black.

## EXPERIMENTAL EXAMPLE 17

Toner was produced in the same manner as in Experimental example 12 with the exception that 2 pbw boron compound having a volume-average particle size of 3  $\mu\text{m}$  was used.

## EXPERIMENTAL EXAMPLE 18

Toner was produced in the same manner as in Experimental example 12 with the exception that 2 pbw boron compound having a volume-average particle size of 28  $\mu\text{m}$  was used.

## EXPERIMENTAL EXAMPLE 19

Toner was produced in the same manner as in Experimental example 12 with the exception that 8 pbw Regal 330 (Cabot; pH9.0; mean primary particle size: 25 nm) was used as carbon black.

## EXPERIMENTAL EXAMPLE 20

Toner was produced in the same manner as in Experimental example 12 with the exception that 0.3 pbw boron compound was used.

## 14

## EXPERIMENTAL EXAMPLE 21

Toner was produced in the same manner as in Experimental example 12 with the exception that 5.5 pbw boron compound was used.

The amount of boron compound present on the surface of the toner particles was measured as described below; measurement results are shown in Table 2.

First, a surface active agent (n-dodecylbenzene sodium sulfonate) was dissolved in purified water and the solution was introduced into a jar with a screw lid, then a weighed toner sample was loaded into the jar and mixed. The material was then filtered to separate the toner from the boron compound dissolved in the solution. The potassium concentration in the solution was assayed via atomic absorption photometry, and the boron compound concentration in the solution was calculated from a previously determined calibration curve. The amount of boron compound present on the surface of the toner particles (wt %) was determined by the equation  $\{(concentration\ of\ boron\ compound\ in\ solution/toner\ concentration\ in\ solvent)\times 100\}$ .

Each of the aforesaid toners were mixed with a pure carrier at a toner-to-carrier weight ratio of 5:95 to produce developer which was used in a digital copier (model Di30; Minolta Co., Ltd.). The toners were evaluated and the evaluation results are shown in Table 2.

## Charge Rise Characteristics

The developer was placed in a plastic bottle and mixed by rotation on a ball mill table at 120 rpm. The charge was measured after 3 min and after 60 min (25° C., 45% RH).

## Post-printing Fog

The aforesaid developers were used to make 20,000 prints using a model Di30 digital copier (Minolta Co., Ltd.), and images were visually examined thereafter. Images with no trace of fog were ranked O, images with slight fog that posed no practical problem were ranked  $\Delta$ , and images with noticeable fog making them unsuitable for practical use were ranked X.

## Post-printing Image Density Irregularity

The aforesaid developers were used to make 20,000 prints using a model Di30 digital copier (Minolta Co., Ltd.), and images were visually examined. Thereafter, 2x2 cm solid images were formed at the four corners and the center of an A4 page, and the reflective density of said images was measured using a MacBeath densitometer. A difference between maximum and minimum image densities of less than 0.05 was ranked O, 0.05 or greater but less than 0.1 was ranked  $\Delta$ , and 0.1 and higher was ranked X.

## Post-printing Dot Reproducibility

The aforesaid developers were used to make 20,000 prints using a model Di30 digital copier (Minolta Co., Ltd.). Thereafter, the fixing temperature was set at 180° C., and a dot image was formed. The dot diameter of the obtained dot image was measured using an image analyzing device to obtain data of about 80~10 dots, and the maximum dot diameter Dmax was determined and ranked. Dmax of less than 185  $\mu\text{m}$  was designated rank 10, 185  $\mu\text{m}$  and higher but less than 187.5  $\mu\text{m}$  was designated rank 9, 197.5  $\mu\text{m}$  and higher but less than 190  $\mu\text{m}$  was designated rank 8, 190  $\mu\text{m}$  and higher but less than 192.5  $\mu\text{m}$  was designated rank 7, 192.5  $\mu\text{m}$  and higher but less than 195  $\mu\text{m}$  was designated rank 6, 195  $\mu\text{m}$  and higher but less than 197.5  $\mu\text{m}$  was designated rank 5. Ranks 9 and 10 are expressed by O, ranks 7 and 8 are expressed by  $\Delta$ , and ranks 6 and below are expressed by X.

TABLE 2

| Amt. on surface (%) | Amt. of charge ( $\mu\text{C/g}$ ) |         | Dot Reproduc- | Density |
|---------------------|------------------------------------|---------|---------------|---------|
|                     | >3 min                             | >60 min |               |         |
| Ex 12               | 0.20                               | -18     | -17           | ○ ○ ○   |
| Ex 13               | 0.07                               | -22     | -24           | ○ ○ ○   |
| Ex 14               | 0.38                               | -17     | -15           | ○ ○ ○   |
| Ex 15               | 0.30                               | -19     | -20           | △ ○ ○   |
| Ex 16               | 0.12                               | -16     | -15           | ○ △ ○   |
| Ex 17               | 0.03                               | -23     | -30           | ○ x x   |
| Ex 18               | 0.60                               | -19     | -11           | x x x   |
| Ex 19               | 0.20                               | -16     | -12           | △ x ○   |
| Ex 20               | 0.04                               | -20     | -26           | ○ ○ x   |
| Ex 21               | 0.52                               | -17     | -10           | x ○ x   |

## EXPERIMENTAL EXAMPLE 22

A mixture of 40 pbw polyester resin L1, 60 pbw polyester resin H1, 2 pbw polyethylene wax (800P; Mitsui Sekiyu Kagaku Kogyo; melt viscosity 5400 cps at 160°C., softening point: 140°C.), 2 pbw polypropylene wax (TS-200; Sanyo Kasei Kogyo; melt viscosity of 120 cps at 160°C., softening point: 145°C.; acid value: 3.5 KOHmg/g), 8 pbw acidic carbon black (Mogul L; Cabot; pH2.5, mean primary particle size: 24 nm), and 2 pbw negative charge controller having the chemical structural formula below



were added to a Henschel mixer and thoroughly mixed. The obtained mixture was fusion kneaded using a twin-shaft extrusion kneader, then cooled. The cooled mixture was coarsely pulverized using a hammer mill, and the coarsely pulverized material was finely pulverized using a jet mill, and then the material was then classified to obtain toner particles having a volume-average particle size of 7.5  $\mu\text{m}$ .

These toner particles were mixed with 0.4 percent-by-weight hydrophobic silica microparticles having a BET specific surface area of 140  $\text{m}^2/\text{g}$  (H2000; Hoechst), and 0.1 percent-by-weight hydrophobic titanium dioxide microparticles having a BET specific surface area of 110  $\text{m}^2/\text{g}$  (STT30A; Chitan Kogyo) to obtain the end toner. The additive exterior microparticles of the toner had a total specific surface area of 67  $\text{m}^2/\text{g}$ .

## EXPERIMENTAL EXAMPLE 23

Toner was produced in the same manner as in Experimental example 22 with the exception that the amount of added hydrophobic silica microparticles was changed to 0.3 wt %, and the amount of added hydrophobic titanium dioxide microparticles was changed to 0.05 wt %. The additive exterior microparticles of the toner had a total specific surface area of 47.5  $\text{m}^2/\text{g}$ .

## EXPERIMENTAL EXAMPLE 24

Toner was produced in the same manner as in Experimental example 22 with the exception that the amount of

added-hydrophobic silica microparticles was changed to 0.3 wt %, and the amount of added hydrophobic titanium dioxide microparticles was changed to 0.4 wt %. The additive exterior microparticles of the toner had a total specific surface area of 86  $\text{m}^2/\text{g}$ .

## EXPERIMENTAL EXAMPLE 25

Toner was produced in the same manner as in Experimental example 22 with the exception that the amount of added hydrophobic silica microparticles was changed to 0.5 wt %, and the amount of added hydrophobic titanium dioxide microparticles was changed to 0.4 wt %. The additive exterior microparticles of the toner had a total specific surface area of 114  $\text{m}^2/\text{g}$ .

## EXPERIMENTAL EXAMPLE 26

Toner was produced in the same manner as in Experimental example 22 with the exception that the amount of added hydrophobic titanium dioxide microparticles was changed to 0.05 wt %. The additive exterior microparticles of the toner had a total specific surface area of 61.5  $\text{m}^2/\text{g}$ .

## EXPERIMENTAL EXAMPLE 27

Toner was produced in the same manner as in Experimental example 22 with the exception that the added hydrophobic silica was changed to 0.1 wt % TS500 (Cabot; BET specific surface area: 225  $\text{m}^2/\text{g}$ ), and the amount of added hydrophobic titanium dioxide microparticles was changed to 0.5 wt %. The additive exterior microparticles of the toner had a total specific surface area of 77.5  $\text{m}^2/\text{g}$ .

## EXPERIMENTAL EXAMPLE 28

Toner was produced in the same manner as in Experimental example 22 with the exception that the amount of added hydrophobic titanium dioxide microparticles was changed to 0.1 wt % anatase titanium dioxide (BET specific surface area: 50  $\text{m}^2/\text{g}$ ) having a mean primary particle size of 50 nm and subjected to hydrophobic processing with n-butytrimethoxysilane. The additive exterior microparticles of the toner had a total specific surface area of 61  $\text{m}^2/\text{g}$ .

## EXPERIMENTAL EXAMPLE 29

Toner was produced in the same manner as in Experimental example 22 with the exception that hydrophobic titanium dioxide was not added. The additive exterior microparticles of the toner had a total specific surface area of 56  $\text{m}^2/\text{g}$ .

## EXPERIMENTAL EXAMPLE 30

Toner was produced in the same manner as in Experimental example 24 with the exception that hydrophobic silica was not added. The additive exterior microparticles of the toner had a total specific surface area of 44  $\text{m}^2/\text{g}$ .

## EXPERIMENTAL EXAMPLE 31

Toner was produced in the same manner as in Experimental example 22 with the exception that 0.4 wt % R809 (Nippon Aerosil; BET specific surface area: 50  $\text{m}^2/\text{g}$ ) was added as the hydrophobic silica. The additive exterior microparticles of the toner had a total specific surface area of 56  $\text{m}^2/\text{g}$ .

## EXPERIMENTAL EXAMPLE 32

Toner was produced in the same manner as in Experimental example 22 with the exception that the amount of

added hydrophobic silica was changed to 1.0 wt %, and the amount of added hydrophobic titanium dioxide was changed to 0.1 wt %. The additive exterior microparticles of the toner had a total specific surface area of 151 m<sup>2</sup>/g.

#### EXPERIMENTAL EXAMPLE 33

Toner was produced in the same manner as in Experimental example 22 with the exception that the amount of added hydrophobic silica was changed to 0.2 wt %, and the amount of added hydrophobic titanium dioxide was changed to 0.05 wt % RX50 (Nippon Aerosil; BET specific surface area: 30 m<sup>2</sup>/g). The additive exterior microparticles of the toner had a total specific surface area of 31 m<sup>2</sup>/g.

#### EXPERIMENTAL EXAMPLE 34

Toner was produced in the same manner as in Experimental example 27 with the exception that the amount of added hydrophobic silica was changed to 0.2 wt %, and the amount of added hydrophobic titanium dioxide was changed to 1.0 wt %. The additive exterior microparticles of the toner had a total specific surface area of 155 m<sup>2</sup>/g.

#### EXPERIMENTAL EXAMPLE 35

Toner was produced in the same manner as in Experimental example 27 with the exception that the amount of added hydrophobic silica was changed to 0.4 wt %, and the amount of added hydrophobic titanium dioxide was changed to 0.5 wt %. The additive exterior microparticles of the toner had a total specific surface area of 145 m<sup>2</sup>/g.

#### EXPERIMENTAL EXAMPLE 36

Toner was produced in the same manner as in Experimental example 26 with the exception that azo dye T77 (Hodogaya Kagaku) was used as a negative charge controller. The additive exterior microparticles of the toner had a total specific surface area of 67 m<sup>2</sup>/g.

#### EXPERIMENTAL EXAMPLE 37

Toner was produced in the same manner as in Experimental example 26 with the exception that calix arene compound E89 (Orient Chemical Industries) was used as a negative charge controller. The additive exterior microparticles of the toner had a total specific surface area of 67 m<sup>2</sup>/g.

#### EXPERIMENTAL EXAMPLE 38

Toner was produced in the same manner as in Experimental example 22 with the exception that quaternary ammonium salt with fluoride VP434 (Hoechst) was used as a negative charge controller. The additive exterior microparticles of the toner had a total specific surface area of 67 m<sup>2</sup>/g.

#### EXPERIMENTAL EXAMPLE 39

Toner was produced in the same manner as in Experimental example 22 with the exception terpene diphenol compound YP90 (Yasuhara Chemicals) was used as a negative charge controller. The additive exterior microparticles of the toner had a total specific surface area of 67 m<sup>2</sup>/g.

The aforesaid toners were evaluated and the evaluation results are shown in Table 3.

#### Toner Flow Characteristics

The apparent specific gravity of each toner was measured using a power tester (Hosokawa Micron). An apparent specific gravity of 0.42 cc/g and higher was ranked O, 0.38

cc/g and higher but less than 0.42 cc/g was ranked Δ, and less than 0.38 cc/g was ranked X.

#### Environmental Resistance

Each of the aforesaid toners were mixed with a pure carrier at a toner-to-carrier weight ratio of 5:95 to produce developer which was used in a digital copier (model Di30; Minolta Co., Ltd.).

Each toner was subjected to charge measurements under conditions of high temperature and high humidity (H/H; 30°C., 85% RH), and low temperature and low humidity (L/L; 10°C., 15% RH). An absolute value of the difference in the H/H and L/L charges of less than 10 μC was ranked O, a value of 10 μC and higher but less than 15 μC was ranked Δ, and a value of 15 μC or higher was ranked X.

#### Transfer Characteristics

Each of the aforesaid developers was used to make 30,000 printings using a model Di30 digital copier (Minolta Co., Ltd.), and the images were visually inspected. An image without loss due to insufficient transfer was ranked O, slight image loss which posed not practical problem was ranked Δ, and serious image loss unsuitable for practical use was ranked X.

#### Charge Rise Characteristics

Each of the aforesaid developers was loaded in a plastic bottle and rotated at 120 rpm on a ball mill table to mix for 5, 10, 30, 60, 120, and 780 minutes, after which the amount of charge was measured (under environmental conditions of 25°C., 45% RH).

The amount of charge after 5 min relative to a maximum charge value {(amount of charge after 5 min/maximum charge value) × 100} of 90% or greater was deemed an extraordinary excellent charge rise and designated by a rank of O, 80% and higher but less than 90% was deemed suitable for practical use and designated by a rank of Δ, and less than 80% was deemed unsuitable for practical use and designated by a rank of X.

#### Initial Fog and Post-printing Fog

Each of the developers was used to make 100,000 prints using a model Di30 digital copier, and the images were visually examined at initial printing (after 100 sheets) and at the end of printing. Images with no trace of fog were ranked O, images with slight fog that posed no practical problem were ranked Δ, and images with noticeable fog making them unsuitable for practical use were ranked X.

TABLE 3

|       | Flow | Environmental Resistance | Transfer | Charge Rise | Initial Fog | Post-print Fog |
|-------|------|--------------------------|----------|-------------|-------------|----------------|
| Ex 22 | ○    | ○                        | ○        | ○           | ○           | ○              |
| Ex 23 | Δ    | ○                        | ○        | ○           | ○           | ○              |
| Ex 24 | Δ    | ○                        | ○        | ○           | ○           | ○              |
| Ex 25 | ○    | ○                        | ○        | ○           | ○           | Δ              |
| Ex 26 | ○    | Δ                        | ○        | ○           | ○           | ○              |
| Ex 27 | Δ    | ○                        | ○        | ○           | ○           | ○              |
| Ex 28 | ○    | Δ                        | ○        | ○           | ○           | ○              |
| Ex 29 | ×    | Δ                        | Δ        | ○           | ○           | ○              |
| Ex 30 | ×    | ○                        | ×        | ○           | ○           | ○              |
| Ex 31 | ×    | ○                        | Δ        | ○           | Δ           | ×              |
| Ex 32 | ○    | ×                        | ○        | ○           | ×           | ×              |
| Ex 33 | ×    | Δ                        | ×        | ○           | Δ           | ×              |
| Ex 34 | Δ    | ○                        | ○        | ○           | ×           | ×              |
| Ex 35 | ○    | Δ                        | ○        | Δ           | Δ           | ×              |
| Ex 36 | ○    | Δ                        | ○        | ×           | ○           | Δ              |
| Ex 37 | ○    | ○                        | ○        | ×           | ×           | ×              |
| Ex 38 | ○    | ○                        | ○        | ×           | Δ           | ×              |
| Ex 39 | ○    | ○                        | ○        | ×           | Δ           | ×              |

What is claimed is:

1. A negatively chargeable toner for developing electrostatic latent images comprising:

negatively chargeable toner particles including a binder resin, a carbon black, an boron compound; said binder resin including a polyester resin and having an acid value of 5 to 50 KOHmg/g, said carbon black having a pH of 1 to 6, and said boron compound represented by a structural formula (A):



wherein  $R_1$  and  $R_3$  respectively represent substituted or non-substituted aryl group,  $R_2$  and  $R_4$  respectively represent hydrogen atom, alkyl group, substituted or non-substituted aryl group,  $X$  represents a cation, and  $n$  is an integer of either 1 or 2.

2. The negatively chargeable toner of claim 1, wherein an amount of the carbon black is from 6 to 12 parts by weight per 100 parts by weight of the binder resin.

3. The negatively chargeable toner of claim 1, wherein the carbon black has a mean primary particle size of 10 to 40 nm.

4. The negatively chargeable toner of claim 1, wherein an amount of the boron compound is from 0.5 to 5 parts by weight per 100 parts by weight of the binder resin.

5. The negatively chargeable toner of claim 1, wherein an amount of the boron compound existing on the surface of the toner particles is from 0.05 to 0.4 percent by weight on the basis of the toner particles.

6. The negatively chargeable toner of claim 1, wherein the binder resin comprises a first resin and a second resin, said first resin having a softening point of 95° to 120° C. and a glass transition point of 50° to 75° C., and said second resin having a softening point of 130° to 160° C. and a glass transition point of 50° to 75° C.

7. The negatively chargeable toner of claim 6, wherein a weight ratio of the first resin to the second resin is 7:3 to 2:8.

8. The negatively chargeable toner of claim 6, wherein the first resin comprises a polyester resin obtained by a polyvalent alcohol component and a polyvalent carboxylic acid component, said polyester resin comprising a bisphenol-A alkylene oxide additive as the polyvalent alcohol component and at least one polyvalent carboxylic acid monomer selected from the group consisting of a terephthalic acid, a fumaric acid, a dodecenylic acid and a benzenetricarboxylic acid as the polyvalent carboxylic acid component.

9. The negatively chargeable toner of claim 6, wherein the first resin comprises a linear polyester resin obtained by a bivalent alcohol component and a bivalent carboxylic acid component.

10. The negatively chargeable toner of claim 6, wherein the second resin comprises a polyester resin obtained by a polyvalent alcohol component and a polyvalent carboxylic acid component, said polyester resin comprising a bisphenol-A alkylene oxide additive as the polyvalent alcohol component and at least one polyvalent carboxylic acid monomer selected from the group consisting of a terephthalic acid, a fumaric acid, a dodecenylic acid and a benzenetricarboxylic acid as the polyvalent carboxylic acid component.

11. The negatively chargeable toner of claim 6, wherein the second resin comprises a polyester resin and a vinyl resin.

12. The negatively chargeable toner of claim 11, wherein the second resin is obtained by a raw monomer of the

polyester resin, a raw monomer of the vinyl resin and a dual-reactive monomer, said dual-reactive monomer being a raw monomer that is able to use dual reactions of a condensation polymerization and a radical polymerization.

13. The negatively chargeable toner of claim 12, wherein the dual-reactive monomer has a carboxyl group and a vinyl group.

14. The negatively chargeable toner of claim 11, wherein an amount of the vinyl resin of the second resin is from 5 to 40 percent by weight on the basis of the second resin.

15. The negatively chargeable toner of claim 1, comprising a wax being contained in an amount of 0.5 to 5 parts by weight per 100 parts by weight of the binder resin.

16. The negatively chargeable toner of claim 1, comprising magnetic particles being contained in an amount of 0.5 to 10 parts by weight per 100 parts by weight of the binder resin.

17. A negatively chargeable toner for developing electrostatic latent images comprising:

negatively chargeable toner particles including a binder resin having an acid value of 5 to 50 KOHmg/g, a colorant, and a boron compound represented by a structural formula (A):



wherein  $R_1$  and  $R_3$  respectively represent substituted or non-substituted aryl group,  $R_2$  and  $R_4$  respectively represent hydrogen atom, alkyl group, substituted or non-substituted aryl group,  $X$  represents a cation, and  $n$  is an integer of either 1 or 2; and

and exterior additive particles adhered to the toner particle surface, said exterior additive particles comprising hydrophobic silica particles and hydrophobic titanium dioxide particles, wherein the additive weight ratio of said hydrophobic silica particles and hydrophobic titanium dioxide particles is within a range of 10:1 to 1:10, a total specific surface area  $S$  of the exterior additive particles is 40 to 130 expressed by the equation (1):

$$S = S_s \times V_s + S_t \times V_t \quad (1)$$

Wherein  $S_s$  is a specific surface area of the hydrophobic silica particles ( $m^2/g$ ),  $V_s$  is an additive amount of hydrophobic silica particles relative to the toner particles (percent-by-weight),  $S_t$  is a specific surface area of the hydrophobic titanium dioxide particles ( $m^2/g$ ), and  $V_t$  is an additive amount of hydrophobic titanium dioxide particles relative to the toner particles (percent-by-weight).

18. The negatively chargeable toner of claim 17, wherein an amount of the boron compound is from 0.5 to 5 parts by weight per 100 parts by weight of the binder resin.

19. The negatively chargeable toner of claim 17, wherein the hydrophobic silica particles have the specific surface area of 100 to 250  $m^2/g$ .

20. The negatively chargeable toner of claim 17, wherein the hydrophobic titanium dioxide particles have the specific surface area of 40 to 150  $m^2/g$ .

21. The negatively chargeable toner of claim 17, wherein said additive weight ratio is within a range of 8:1 to 1:5, and said total specific surface area  $S$  is 50 to 100.

22. The negatively chargeable toner of claim 17, wherein the colorant is a carbon black having a pH value of 1 to 6.

21

23. The negatively chargeable toner of claim 22, wherein an amount of the carbon black is from 6 to 12 parts by weight per 100 parts by weight of the binder resin.

24. The negatively chargeable toner of claim 22, wherein the carbon black has a mean primary particle size of 10 to 40 nm.

25. The negatively chargeable toner of claim 17, wherein the binder resin comprises a first resin and a second resin, said first resin having a softening point of 95° to 120° C. and a glass transition point of 50° to 75° C., and said second resin having a softening point of 130° to 160° C. and a glass transition point of 50° to 75° C.

26. The negatively chargeable toner of claim 25, wherein a weight ratio of the first resin to the second resin is 7:3 to 2:8.

27. The negatively chargeable toner of claim 25, wherein the first resin comprises a polyester resin obtained by a polyvalent alcohol component and a polyvalent carboxylic acid component, said polyester resin comprising a bisphenol-A alkylene oxide additive as the polyvalent alcohol component and at least one polyvalent carboxylic acid monomer selected from the group consisting of a terephthalic acid, a fumaric acid, a dodecenylsuccinic acid and a benzenetricarboxylic acid as the polyvalent carboxylic acid component.

28. The negatively chargeable toner of claim 25, wherein the first resin comprises a linear polyester resin obtained by a bivalent alcohol component and a bivalent carboxylic acid component.

29. The negatively chargeable toner of claim 25, wherein the second resin comprises a polyester resin obtained by a polyvalent alcohol component and a polyvalent carboxylic

22

acid component, said polyester resin comprising a bisphenol-A alkylene oxide additive as the polyvalent alcohol component and at least one polyvalent carboxylic acid monomer selected from the group consisting of a terephthalic acid, a fumaric acid, a dodecenylsuccinic acid and a benzenetricarboxylic acid as the polyvalent carboxylic acid component.

30. The negatively chargeable toner of claim 25, wherein the second resin comprises a polyester resin and a vinyl resin.

31. The negatively chargeable toner of claim 30, wherein the second resin is obtained by a raw monomer of the polyester resin, a raw monomer of the vinyl resin and a dual-reactive monomer, said dual-reactive monomer being a raw monomer that is able to use dual reactions of a condensation polymerization and a radical polymerization.

32. The negatively chargeable toner of claim 31, wherein the dual-reactive monomer has a carboxyl group and a vinyl group.

33. The negatively chargeable toner of claim 30, wherein an amount of the vinyl resin of the second resin is from 5 to 40 percent by weight on the basis of the second resin.

34. The negatively chargeable toner of claim 17, comprising a wax being contained in an amount of 0.5 to 5 parts by weight per 100 parts by weight of the binder resin.

35. The negatively chargeable toner of claim 17, comprising magnetic particles being contained in an amount of 0.5 to 10 parts by weight per 100 parts by weight of the binder resin.

\* \* \* \* \*

UNITED STATES PATENT AND TRADEMARK OFFICE  
**CERTIFICATE OF CORRECTION**

PATENT NO. : 5,776,647  
DATED : July 7, 1998  
INVENTOR(S) : Kenichi Kido, et al.

It is certified that error appears in the above-identified patent and that said Letters Patent is hereby corrected as shown below:

Col. 21, line 18, change "apolyvalent" to -- polyvalent --

Signed and Sealed this  
Twenty-third Day of February, 1999

Attest:



Q. TODD DICKINSON

*Attesting Officer*

*Acting Commissioner of Patents and Trademarks*